

June 10, 1941.

E. F. VON ENDE ET AL  
METHOD OF PRODUCING VENEERS

2,245,170

Filed Aug. 18, 1937

Fig. 1



Fig. 4



Fig. 2



Fig. 3



Fig. 5



Fig. 7



Fig. 8



Fig. 6



Inventor:  
Emil von Ende  
Heinrich Geffcken

By *Paul Klem*  
Attorney

## UNITED STATES PATENT OFFICE

2,245,170

## METHOD OF PRODUCING VENEERS

Emil Freiherr von Ende, Haslach L/K., and  
Heinrich Geffcken, Berlin, GermanyApplication August 18, 1937, Serial No. 159,734  
In Germany March 6, 1937

3 Claims. (Cl. 41—35)

The present invention relates to improvements in artificially veined veneers and a method of making the same, more particularly to veneers of the type obtained by gluing together under heat a plurality of superposed ordinary veneers in a press having profiled, such as corrugated, dies, and by subsequently cutting up the composite block thus obtained into new veneers along cutting lines intersecting the initial veneers in the block.

In carrying out the aforescribed method, difficulties have been encountered in that the fibres in the finished veneer were torn or splintered or the veneer easily broken or cracked. Moreover, if the veneer thus obtained was glued upon a base, the glue easily penetrated through the veneer, producing stains and spoiling the polish thereon.

By the present invention the above drawbacks are substantially overcome by the employment of special veneers for producing the intermediate blocks in the manufacturing process and a novel compressing operation in forming the composite intermediate block from which the final veneers are cut.

With this and other objects in view, the invention contemplates the use of so-called pared-off veneers obtained by spirally cutting a trunk from the outside to the inside in place of the usual veneers obtained by transverse cutting or sawing in planes more or less parallel to the axis of the trunk. A block or stack of pared-off veneers of this type is then subjected to pressure, preferably in such a manner that the pressure is applied at first to one side only of the stack and gradually increased and extended until covering the entire stack area. It was found in carrying out the above process that pared-off veneers are better able to stand the tensile and compressive forces exerted thereon during compression, thereby preventing tearing or breaking as experienced with the ordinary type of veneer used in the prior art processes. Moreover, pared-off veneers have the advantage of gliding upon one another more easily and smoothly if subjected to pressure in a press with profiled dies thereby enabling them to become deformed more easily and to conform and accommodate themselves to the shape of the pressing dies without tearing or splintering. These properties are apparently due to the fact that adjacent cells or fibres in pared-off or spirally cut veneers belong to the same period of growth (annual rings) while in the case of transversely cut veneers cells of successive periods of growth hav-

ing different mechanical properties lie side by side.

The above and further objects and advantages of the invention will become more apparent from the following detailed description of a method and means for carrying out the invention taken with reference to the accompanying drawing forming part of this specification and wherein:

Figure 1 shows for the sake of illustration the production of spirally cut or pared-off veneers for use with the invention;

Figures 2 and 3 illustrate diagrammatically pressing devices suitable for carrying out the invention;

Figure 4 is a partial section on an enlarged scale of a compressed block of veneers ready for cutting into final veneers;

Figure 5 illustrates a surface pattern of a veneer obtained by the invention;

Figure 6 shows a plurality of veneers stacked before compressing according to a modification of the invention;

Figure 7 illustrates another modification of the invention; and

Figure 8 shows the surface of a finished veneer obtained by the modified processes according to Figures 6 and 7.

Similar reference numerals identify similar parts throughout the different views of the drawing.

Referring to Figure 1, this illustrates the cutting or paring off of a veneer sheet from a trunk 1 by means of paring knife 2 whereby the veneer obtained contains cells or fibres of the same annual rings originating from the same annual rings of a trunk pertaining to the same period of growth and having substantially uniform mechanical and other properties.

A veneer sheet obtained in this manner is cut into suitable elements which may be freed from moisture and subjected to the action of a mordant in the usual manner and/or dyed if desired and are then surfaced with a gluing substance. The elements or sheets thus prepared are then piled upon each other to form a stack and the stack placed in a press of the type as shown in Figure 2. The latter consists of a frame 3 carrying a lower plate or block 4 having secured thereto a die 6 formed with a profiled, such as a corrugated, face as shown in the example illustrated. The press further comprises an upper block 5 with a die 8 having a similar profile or cross-section to the die 6 of the lower pressing block. The stack 7 of veneers assembled in the above described manner

is placed upon the lower die 6 and the upper section moved in a downward direction indicated by the arrow 11 in a manner well understood. There is further shown a wedge-like member 9 of rubber or other yielding material placed between the upper face of the stack and the adjacent upper die plate 8. In the drawing the thickness of the member 9 has been shown on an exaggerated scale for clarity of illustration. There is furthermore provided a suitable heating system or furnace indicated at 10 surrounding the die sections and block 7 placed therebetween.

In carrying out the pressing operation, the block 7 is at first heated to a suitable temperature, whereupon the press is closed to apply increasing pressure to the stack. The effect of the wedge-shaped rubber member 9 is to cause the pressure to be initially applied to the block 7 at the left-hand side only of the stack area and to extend gradually over the entire face of the block or stack as the die 8 is moved towards the stack and the pressure increased. Owing to the pliability of the pared-off veneers in the stack 7 and to the uniform properties of the cells or fibres within the individual veneers, the latter will offer relatively small resistance and glide easily and smoothly upon one another during the pressing operation thereby conforming and accommodating themselves readily to the shape of the dies 6 and 8. After the compression the temperature is suitably adjusted and the block allowed to set and thereafter to cool in the press.

Figure 3 shows a modified arrangement of a press wherein the wedge-shaped resilient member 13 is placed between the die member 12 and the upper section or block 5. This arrangement has the advantage that the plate 13 may be protected against excessive heat by cooling the die 5. It is furthermore possible by this arrangement to lift the die 5 after the block has been preliminarily compressed to remove the wedge 13 and thereafter to re-compress the stack in order to preserve the wedge 13 and prevent it from being subjected to excessive and prolonged heating. A further advantage is the fact that in this manner the wedge 13 can be more easily removed from the stack and is not affected by or soiled with glue as in the case of the arrangement shown in Figure 2.

Figure 4 shows on an enlarged cross-section, a portion of a finished veneer block obtained after gluing and compressing in the manner described hereinbefore. This block is then cut into new veneers along parallel lines as indicated by  $x-y$  intersecting the initial veneers whereby the veneers obtained in this manner exhibit artificial veins such as shown in Figure 5. These veins will be especially impressive if the individual veneer sheets in the block 7 originated from different kinds of wood or are tainted with different colors and are arranged in suitable succession within the block.

The veneers made in the above-described manner are generally free from knot holes. In most cases this constitutes an advantage but there are cases where a knot hole or "bird's-eye" appearance of the final veneer is desired. This can be obtained in a simple and easy manner in the manufacture of artificial veneers in accordance with the process of the present invention such as described in the following with reference to Figures 6 and 8.

In Figure 6 there is shown a stack 7 of veneers prior to compression with wooden beads 14

strewn irregularly between the individual veneers. If the beads are of suitable size and of a flattened or lentile-like shape, they will be completely embedded in the veneer block during the compressing operation. By cutting such a block in the manner described, final veneers are obtained having an appearance with "bird's-eye" effects as shown in Figure 8 similar to the patterns characteristic of certain natural knotty or curly woods. In the making of veneers of this type, the press is preferably designed in such a manner that the profiled dies 6 and 8 fit into each other exactly such as in the case of corrugated dye blocks as shown in Figure 2.

15 A similar effect may be obtained by preliminarily producing blocks of corrugated veneers of substantially smaller thickness, perforating the same, and driving wooden pegs into the perforations to hold the blocks together as shown in Figure 7. A plurality of such blocks may then be piled upon one another and glued together and compressed to form a larger block in the manner as will be understood from the above. Preferably the temperature during the second compressing operation in uniting the preformed blocks is higher than the temperature employed in forming the initial blocks. The preliminary pressing of the smaller blocks into the final corrugated shape of the sheets as shown in Figure 7 has the effect to prevent tearing of the sheets when driving the peg 16 into the perforations 15. If a block of this type is divided into veneers by parallel saw cuts in the manner described, a knotty or "bird's-eye" appearance is obtained 30 in a similar manner as hereinbefore described and shown in Figure 8.

It will be evident from the above that the invention is not limited to the specific arrangements and methods described herein for illustration 40 but that the underlying inventive idea is susceptible of various modifications and embodiments coming within the broader scope of the invention as defined in the appended claims.

We claim:

45 1. The method of producing artificially veined wooden veneer comprising the steps of stacking a plurality of glue surfaced initial pared-off veneer sheets having fibres belonging to the same period of growth of a trunk, heating and initially pressing a limited rim portion of the stack, increasing and gradually extending the pressure until covering the entire stack area, to deform the individual sheets out of their original planar surface, allowing the stack to cool and set into a block, driving wooden pegs through said block 50 transversely to said sheets, and cutting said block into final veneers.

55 2. In a method of producing artificially veined wooden veneers by transversely cutting a consolidated block of initial sheets of pared-off veneers each consisting of fibres belonging to substantially the same period of growth of a trunk, the steps of heating a stack of initial glue-surfaced pared-off veneer sheets, initially compressing a limited marginal portion of the stack area to deform the individual sheets into a corrugated shape out of their initial planar shape, progressively increasing and extending the deforming pressure until covering the entire stack area, allowing the stack to cool and set into a block, and transversely cutting said block into final veneer sheets.

60 3. The method of producing artificially veined wooden veneer comprising the steps of stacking a plurality of glue surfaced initial sheets of

pared-off veneer belonging to the same period of growth of a trunk, while simultaneously strewing wooden beads between adjacent sheets of the stack, heating and initially pressing a limited rim portion of the stack, increasing and 5 gradually extending the pressure until covering

the entire stack area, thereby to deform the individual sheets out of their original planar surface, allowing the stack to cool and set into a block, and cutting said block into final veneers.

EMIL FREIHERR VON ENDE.  
HEINRICH GEFFCKEN.